

3,788,857

**METHOD OF INCORPORATING PHOTOGRAPHIC ADJUVANTS INTO HYDROPHILIC COLLOIDS**

Raphael Karel Van Poucke, Berchem, and Robert Joseph Pollet, Vremde, Belgium, assignors to Agfa-Gevaert N.V., Mortsel, Belgium

No Drawing. Filed June 4, 1971, Ser. No. 150,214  
Claims priority, application Great Britain, Aug. 13, 1970,

39,116/70

Int. Cl. G03c 1/40

U.S. CL. 96—100

16 Claims

**ABSTRACT OF THE DISCLOSURE**

A photographic chemical adjvant is incorporated into a hydrophilic colloid composition by dispersing a solution of the chemical adjvant in the hydrophilic colloid composition in the presence of a high-boiling substantially water-insoluble aliphatic alcohol or ethoxylated derivative thereof which corresponds to the formula:



wherein

$n$  is 0 or 1 and  $m$  is 0 to 30,

$\text{R}_3$  is hydrogen or when  $n$  is 1 may be alkyl, and each of  $\text{R}_1$  and  $\text{R}_2$  stands for a straight-chain or branched-chain alkyl group or together represent the atoms necessary to complete an aliphatic ring structure,  $\text{R}_1$  and  $\text{R}_2$  together comprising at least 5 carbon atoms.

The colloid composition can be a light-sensitive silver halide emulsion or a non-light sensitive water-permeable colloid composition. The high boiling alcohols or ethoxylated derivatives thereof have the particular advantage of reducing the viscosity of the colloid compositions and maintaining the viscosity at a stable level.

The present invention is concerned with the use of high-boiling substantially water-insoluble aliphatic alcohols or ethoxylated derivatives thereof in dispersing chemical adjvants into hydrophilic colloids employed in the formation of photosensitive and even non-photosensitive layers of photographic silver halide elements.

In the manufacture of a photographic material numerous adjvants should be brought into operative association in one or more of the hydrophilic colloid layers of the said material. These adjvants include amongst others color couplers, competing couplers, mask-forming compounds, dyes e.g. filter dyes, antihalation dyes and sensitizing dyes, stabilizers, U.V. -absorbers, optical brightening agents, etc.

The methods according to which these adjvants are incorporated into the photographic hydrophilic colloid layers present numerous problems and much effort has been directed to solve these problems, particularly with regard to the incorporation in photographic emulsions of color couplers and mask-forming compounds.

By color coupler is meant any compound which in silver halide photography couples with an oxidized aromatic primary amino color developing agent to form a dye image. By mask-forming compound is meant a compound which oxidatively couples with a color coupler in an oxidizing bleaching bath as for example described in British Pats. Nos. 880,862 and 975,932 to form a colored mask image.

For various reasons it is desirable that the chemical adjvants when incorporated in photographic photosensitive or non-photosensitive layers of a photographic silver halide element remain immobile in the layer in which they

have been incorporated. For instance color couplers and mask-forming compounds should not wander or diffuse through the photosensitive silver halide emulsion from their original site otherwise color separation will be imperfect and result in final dye images that are degraded.

5 A common method employed to render chemical adjvants e.g. color couplers and mask-formers non-diffusible in hydrophilic colloid media is to provide them in the course of their synthesis with one or more ballast groups, e.g. a long straight-chain or branched-chain aliphatic group such as an alkyl or alkylene group comprising from 5 to 20 carbon atoms. The presence of this ballast group imparts to the molecule a hydrophobic character and therefore, these non-diffusible color couplers and mask-

10 formers are generally also provided with one or more salt-forming groups e.g. carboxy groups and preferably sulpho groups, so that these compounds can be dissolved in the photographic emulsions in the form of their soluble alkali salts.

20 However, the incorporation of these non-diffusible adjvants containing salt-forming groups, into aqueous hydrophilic colloid compositions frequently poses a number of difficulties. For instance, some compounds are soluble only in highly alkaline solutions, which might give rise 25 to hydrolysis of possibly present ester groups or which are too basic for use as such in conventional photosensitive silver halide material since high pH-values give rise to fogging of the emulsion. Therefore, the hydrophilic colloid composition should be reacidified afterwards 30 whereby flocculation might occur and whereby inorganic salts are formed.

35 Alternate processes of incorporating chemical adjvants e.g. color couplers in photographic colloids make use of dispersion techniques. One of the advantages of these techniques is that couplers may be used which are water-insoluble and contain no salt-forming groups.

40 According to one of said dispersion techniques the couplers are dissolved in water-immiscible, oily type solvents or "crystalloids" such as tricresyl phosphate and di-n-butyl phthalate and the resulting solution added to an aqueous phase containing a dispersing agent such as gelatin or a higher fatty alcohol sulphate. The mixture is then passed through a homogenizing apparatus wherein 45 is formed a dispersion of the oily coupler solution in the aqueous medium. In some instances, the dissolution of the coupler in the oily solvent is facilitated by the use of an auxiliary low-boiling water-immiscible solvent which is subsequently removed by evaporation. The above dispersion of coupler is then mixed with a gelatino silver halide 50 emulsion and coated in the usual manner to produce a system in which particles of coupler, surrounded by an oily membrane, are distributed throughout the gel matrix.

55 In this dispersion technique difficulties are sometimes encountered in that the coupler, owing to the limited solvent action of the oily type solvent used, has the tendency to crystallize in the emulsion. This crystallization of the coupler is undesirable because the coupler reacts less readily in the color-forming reaction when crystalline and therefore yields less dye. Another difficulty sometimes encountered in this dispersion technique is that this procedure does not always produce dispersions of sufficiently small particle size with the result that the sharpness of the photographic images suffers.

60 A new dispersion technique has now been found for incorporating chemical adjvants into photographic hydrophilic colloid coating compositions for forming water-permeable colloid layers of a photo-sensitive silver halide element, which new technique does not show the disadvantages of the above dispersion technique.

65 Though this new method may be employed with particular advantage to introduce non-diffusing color couplers

and mask-formers into photographic photosensitive emulsions it can also be used to introduce into photo-sensitive emulsions other photographic emulsion auxiliary compounds such as competing couplers, which are used in color photography as described in British Pat. 861,138, light-screening dyes, sensitizing dyes, stabilizers, etc. Moreover, the method of the present invention can also be employed in the preparation of uniform dispersions of photographic compounds in unsensitized photographic colloid compositions. For example, it may be used in the production of water-permeable intermediate layers in which it is desired uniformly to disperse a light-absorbing filter or antihalation dye, competing couplers and other photographic active substances such as UV-absorbers, optical brightening agents, etc.

The method of the invention may be particularly employed for the incorporation of substantially water-insoluble compounds say compounds of which not more than 3% by weight dissolves in water at room temperature (20%).

(25%). In accordance with the method of the present invention a photographic chemical adjuvant is uniformly distributed throughout a hydrophilic colloid coating composition for forming one of the layers of a photographic silver halide element by dispersing a solution of the said chemical adjuvant in the said photographic hydrophilic colloid coating composition, or, first dispersing the said solution in water or in an aqueous solution of a water-soluble colloid for example gelatin and then mixing the dispersion thus formed with the said hydrophilic colloid coating composition, wherein the said dispersing occurs in the presence of a high-boiling substantially water-insoluble aliphatic alcohol or ethoxylated derivative thereof corresponding to the formula:



wherein:

*n* stands for 0 or 1,

*m* stands for 0 to 30, preferably 0 to 12,

$R_1$  stands for  $C_6H_5$ , preferably  $C_6H_4$ ,  
 $R_3$  stands for hydrogen or when  $n=1$  may be alkyl such as methyl, and  
each of  $R_1$  and  $R_2$  stands for a straight-chain or branched-chain alkyl group or together stand for the atoms necessary to close an alicyclic ring structure,  $R_1$  and  $R_2$  together comprising at least 5 C-atoms.

The resulting coating composition comprises the said colloid having homogeneously distributed therein droplets comprising the chemical adjuvant and the high-boiling alcohol. The high-boiling alcohol is readily penetrated by the photographic developing solution and other processing baths. Photographic color images are produced with high maximum density and excellent sharpness.

One particular advantage of the method of the present invention is that the high-boiling substantially water-insoluble aliphatic alcohol or ethoxylated derivative thereof has a favourable effect on the viscosity of gelatin coating compositions in that the viscosity can be maintained at a stable level. It is known that many chemical adjuvants when incorporated in photosensitive or non-photosensitive hydrophilic colloid compositions cause changes in the viscosity of these compositions when added thereof. The viscosity increases with time so that uniform coating thicknesses cannot be realized. Among the compounds that pose problems as regards keeping the viscosity constant may be mentioned color couplers comprising a carboxyl group. These color couplers cannot be dispersed according to known dispersion techniques into hydrophilic colloid compositions and when dissolved therein from alkaline solutions they require high pH-values in order to prevent flocculation.

A photographic element according to the invention comprises a water-permeable layer having a water-soluble

colloid binder, such as a photo-sensitive gelatino silver halide emulsion layer or a non-photo-sensitive gelatin layer, in which are dispersed droplets comprising a chemical adjuvant and a high-boiling alcohol as defined above.

5 Examples of alcohols corresponding to the above formula are the widely known branched-chain primary oxo-alcohols having at least 8 C-atoms such as isoctyl alcohol, isodecyl alcohol, isotridecyl alcohol, isohexadecyl alcohol and isoctadecyl alcohol. Isooctyl alcohol is a commercial material prepared from  $C_7$ -olefins by means of the oxo-synthesis (cf. H. Römpf, *Chemie Lexikon-Francksche Verlag-Stuttgart*, West Germany), and is a mixture of primary branched-chain  $C_8$ -alcohols. Isodecyl alcohol is a commercial material prepared from  $C_9$ -olefins (tripropylene) by means of the oxo-reaction and is a mixture of primary branched-chain  $C_{10}$ -alcohols. Isotridecyl alcohol is a commercial material prepared from  $C_{12}$ -olefins (triisobutylene, tetrapropylene or di(2-methyl-1-pentene) by means of the oxo-reaction and is a mixture of primary branched-chain  $C_{13}$ -alcohols. Isohexadecyl alcohol and isoctadecyl alcohol are commercial materials prepared by aldol-condensation of  $C_8$  or  $C_9$ -aldehydes formed by oxo-synthesis; isohexadecyl alcohol is a mixture of branched-chain  $C_{16}$ -alcohols mainly consisting of alcohols as represented by the formula:



wherein  $R'$ =dimethyl butyl and  $R''$ =dimethylhexyl whereas isoctadecyl alcohol is a branched-chain alcohol for which the following formula is given:



40 More details regarding the preparation, the composition and the properties of branched-chain oxo-alcohols can be found in *Fortsch. Chem. Forsch.* Bd. 11/1, pp. 121-134 and in the references cited therein.

Other examples of branched-chain alcohols are hydro-  
abietyl alcohol which is an alicyclic alcohol having the  
formula:



the branched-chain commercially available aliphatic secondary alcohols such as isotetradecyl alcohol having the formula:



### and 2-butylacetone

and 2-butyloctanol.

Other branched-chain alcohols suitable for use in the method of the invention are the branched-chain alcohols prepared by alkaline condensation using catalytic amounts of alkali such as potassium hydroxide at temperatures comprised between 200 and 300° C. (known as Guerbet-reaction—see e.g. Fette-Seifen-Anstrichmittel, 71, No. 3, pp. 215-218 (1969)) of a branched-chain or straight-chain alcohol with the same or other branched-chain or straight-chain alcohol.

Other alcohols suitable for use in accordance with the present invention are those having recurring oxyethylene units which can be prepared from the above examples of alcohols by ethoxylation.

The high-boiling alcohols of use in accordance with the present invention are substantially colourless, from light-viscous to heavy viscous liquids at ordinary temperatures. They are inert toward light-sensitive silver halide emulsions and are stable toward light, heat and humidity in addition to being inert to the various processing baths which may be encountered such as developers, oxidized developers, bleach baths, fixing baths, etc. and to the photographic compounds that may be associated with them in the photographic material.

In carrying out the method of the invention, the chemical adjuvants may be dissolved in the high-boiling alcohol whereupon the solution is dispersed directly in the photographic hydrophilic colloid coating composition or—particularly when it is intended to distribute photographic silver halide emulsion auxiliary compounds in a silver halide emulsion ready for coating—first dispersed in water or gelatin solution or in any aqueous colloid which is miscible with the said coating composition, the resulting dispersion then being stored to create stocks of concentrated dispersions from which, whenever required, parts can be taken for addition to hydrophilic colloid coating compositions such as a gelatino silver halide emulsion. The dispersion of the above solution into the aqueous phase may be assisted by the use of high-speed stirrers, homogenizers, colloid mills, ultrasonic wave generators or the like and the dispersions may be stabilized by the addition of emulsifying or dispersing agents.

The dispersion may also be formed by dispersing into an aqueous phase i.e. into water, into a gelatin solution or other aqueous colloid or into the hydrophilic colloid coating composition a solution of chemical adjuvant and the high-boiling alcohol in one or more auxiliary organic solvents, which may be low-boiling substantially water-insoluble organic solvents or appreciably water-soluble organic solvents or a mixture of both, and subsequently removing the said auxiliary solvent from the aqueous phase. It is also possible to add auxiliary solvent(s) to the aqueous phase before dispersing therein the solution comprising chemical adjuvant, high-boiling alcohol and auxiliary solvent(s).

We have referred to dissolving the chemical adjuvant in the said high-boiling alcohol in the presence of an auxiliary solvent or mixture of auxiliary solvents and dispersing the mixture in an aqueous phase after which the auxiliary solvent is removed. Although this is not necessary in the process of the present invention, in many cases it is desirable to proceed in this way using an auxiliary solvent, preferably a low-boiling substantially water-insoluble solvent, which can be removed before coating the hydrophilic colloid coating composition, for instance because in this way, the amount of high-boiling alcohol necessary to dissolve the chemical adjuvant can be reduced markedly.

Low-boiling substantially water-immiscible solvents suitable for use together with the high-boiling alcohol preferably have a solubility in water of at most 25% by weight at room temperature, say 20° C. They preferably have a boiling point of at least 130° C. and a sufficiently high vapor pressure so that they can be removed from the dispersions made by evaporation, if necessary, by applying a vacuum of 500 to 10 mm. Hg at a temperature of 25 to 80° C.

Examples of suitable substantially water-insoluble solvents that may be used in the method of the present invention are: methylene chloride, methyl formate, ethyl formate, n-butyl formate, methyl acetate, ethyl acetate, n-propyl acetate, isopropyl acetate, butyl acetate, methyl propionate, ethyl propionate, carbon tetrachloride, sym-tetrachloroethane, 1,1,2 - trichloroethane, 1,2 - dichloropropane, chloroform, n-butyl alcohol, diethyl ketone,

methyl n-propyl ketone, diisopropyl ether, cyclohexane, methylcyclohexane, benzene, toluene, nitromethane, etc.

When employing in the preparation of the solution of chemical adjuvant and high-boiling alcohol a low-boiling substantially water-immiscible solvent, this solvent is preferably removed during and/or after dispersing the solution into the water, the aqueous colloid or the hydrophilic colloid coating composition. Removal of the said solvent occurs by evaporation, if necessary by applying a reduced pressure, say from 500 mm. to 10 mm. Hg, and/or moderate heating. Of course, it is also possible to leave the low-boiling water-immiscible solvent in the dispersion and to remove it by evaporation on drying the coated hydrophilic colloid composition; this is effected by allowing the solvent to escape on drying the coated composition which is only applicable when sufficiently volatile solvents are used.

It may be interesting in some cases to use together with the high-boiling alcohol and the low-boiling substantially water-insoluble solvent, if employed, an appreciably water-soluble organic solvent examples of which are methanol, ethanol, isopropyl alcohol, dimethyl sulphoxide, tetrahydrofuran, N-methyl - 2 - pyrrolidone, dioxan, dimethyl formamide, dimethoxethane, formamide, ethylene glycol, acetonitrile, acetone, butyrolactone, ethylene glycol monomethyl ether, ethylene glycol monoethyl ether, ethylene glycol monobutyl ether, diethylene glycol monomethyl ether, diacetone alcohol and tetrahydrothiophene-1,1-dioxide.

The water-soluble organic solvents can be removed from the dispersion in the aqueous colloid or from the hydrophilic colloid coating composition—unless this is deemed unnecessary because they have no disadvantageous effect on the physical or photographic properties of the photographic element when left in the dispersion—by washing the chilled and thereby gelled colloid composition. When used in addition to a low-boiling substantially water-insoluble solvent they are removed together with the said low-boiling solvent by evaporation unless they have too high a vapor pressure, in which case they can be removed, if necessary, as indicated above.

As already stated above, in dispersing the solution comprising chemical adjuvant and high-boiling alcohol in the aqueous phase which may be water or an aqueous colloid or a hydrophilic colloid coating composition for forming a layer of a photographic light-sensitive silver halide element, it is desirable to use an emulsifying or dispersing agent.

Though the dispersing or emulsifying agent is generally added to the aqueous phase into which the solution of chemical adjuvant in high-boiling alcohol and auxiliary solvent(s), if employed, is dispersed it is also possible to add said dispersing or emulsifying agent already at the step of dissolving the said chemical adjuvant in the high-boiling alcohol and the auxiliary solvent, if employed.

A survey of dispersing agents and emulsifying agents, representatives of which can be applied in the method of the present invention, is given by Gerhard Gewalek "Wasch- und Netzmittel" Akademieverlag Berlin (1962). Examples of suitable wetting agents are: the sodium salt of N-methyloleyl tauride, sodium stearate, 2-heptadecenylbenzimidazole 5-sulphonic acid sodium salt, sodium sulphonates of higher aliphatic alcohols e.g. 2-methoxyhexanol sodium sulphonate, sodium diisooctyl-sulphosuccinate, sodium dodecyl sulphate, and tetradecyl benzene sulphonic acid sodium salt.

In the method of the present invention wherein high-boiling alcohols corresponding to the above formula are used it was found very interesting to use as dispersing or emulsifying agents ionic surface active compounds derived from alcohols corresponding to the above general formula for example branched-chain aliphatic sulphates, sulphonates, carboxylates, phosphates, etc., which may comprise recurring ethylene oxide units, especially sur-

face active compounds corresponding to the following general formula:



wherein:

*n*,  $R_1$ ,  $R_2$  and  $R_3$  have the same significance as shown, and

$Z$  stands for the groups  $-\text{SO}_3\text{M}$ ,  $-\text{OSO}_3\text{M}$ ,



wherein  $X$  is alkylene, aralkylene or arylene, or the group  $-\text{Y}-\text{A}-\text{SO}_3\text{M}$  wherein  $Y$  is oxygen or sulphur and  $A$  stands for alkylene, substituted alkylene, e.g. alkylene substituted by hydroxyl, or aralkylene,  $M$  being hydrogen, an alkali metal atom such as lithium, sodium and potassium, ammonium or organic ammonium, e.g. diethanol ammonium, triethanol ammonium and morpholinium.

Representative examples of ionic surface active compounds corresponding to the foregoing general formula can be found e.g. in copending applicants Nos. 27,049/70, 27,050/70, 27,080/70 and 27,081/70.

The preferred embodiment of the present invention for incorporating photographic chemical adjuvants into photographic hydrophilic colloid coating compositions comprises the steps of dissolving the said adjuvant in the said high-boiling alcohol and a low-boiling substantially water-insoluble organic solvent e.g. ethyl acetate dispersing the solution formed in the presence of an emulsifying or dispersing agent into water or an aqueous colloid, removing substantially all of the low-boiling substantially water-insoluble organic solvent by evaporation and admixing the resulting dispersion of liquid particles of chemical adjuvant and high-boiling alcohol in water or the aqueous colloid with the hydrophilic colloid coating composition e.g. a photo-sensitive silver halide emulsion.

The amount of high-boiling alcohol used in the method according to the present invention is dependent on the solubility of the particular chemical adjuvant therein and on the optional use of the low-boiling substantially water-insoluble organic solvent or the appreciably water-soluble organic solvent or the mixture of both. This amount can vary within very wide limits but is preferably restricted to a minimum, taking care that the dispersed particles of compound and alcohol in the photographic hydrophilic colloid coating composition for forming a layer of a photographic photosensitive silver halide material are liquid under the conditions of coating and processing the said material. Where in the absence of an auxiliary solvent, the ratio of chemical compound to high-boiling alcohol is generally comprised between 1:10 and 1:1, the amount of said alcohol can be reduced to one part or less than one part per part of chemical compound by the use of an auxiliary solvent, preferably a low-boiling water-immiscible solvent. Therefore, the chemical adjuvant is preferably dissolved in a solvent mixture of such composition that the ratio of chemical adjuvant to high-boiling alcohol will be one part of chemical adjuvant to one part or less than one part of the said high-boiling alcohol, for instance a ratio of chemical adjuvant to high-boiling alcohol comprised between 1:1 and 20:1.

The water or aqueous colloid such as aqueous gelatin into which the solution comprising chemical adjuvant and alcohol can be dispersed prior to admixture with the hydrophilic colloid coating composition preferably comprises a minimum of water in order to obtain dispersions as concentrated as possible which is particularly advantageous for storing purposes.

The amount of stored dispersion to be added to the hydrophilic colloid coating composition for forming a layer of a photographic photo-sensitive silver halide element is such that the chemical adjuvant is present in the resulting

layer in the concentration desired. This amount is naturally dependent on the concentration of the said adjuvant in the said dispersion.

The amount of dispersing agent or emulsifying agent used in making the dispersions in the aqueous phase of photographic compounds according to the method of the present invention, may vary within very wide limit; it is generally comprised between 2 and 30% by weight relative to the weight of adjuvant to be dispersed.

10 Although in applying the method according to the present invention for incorporating chemical adjuvants in hydrophilic colloid media, the use of gelatin as hydrophilic colloid is favoured, other water-soluble colloidal materials or mixtures of them can be used too e.g. colloidal albumin, zein, casein, a cellulose derivative such as carboxymethyl cellulose, a synthetic hydrophilic colloid such as polyvinyl alcohol, poly-N-vinyl pyrrolidone, etc.

15 The following examples illustrate the present invention.

#### EXAMPLE 1

20 1.5 g. of the phenol color coupler having the formula:



25 was dissolved in a mixture of 4.5 ml. of ethyl acetate and 1.5 ml. of isoctadecyl alcohol (commercially available e.g. from Farbwerke Hoechst A.G., Frankfurt am Main, Hochst, West Germany) to which 0.15 g. of sodium isoctadecyl sulphate had been added.

30 The solution formed was admixed by means of a high-speed stirrer with 58 g. of a warm (55° C.) 10% aqueous solution of gelatin. After having homogenized the mixture for 2 minutes, 40 ml. of water heated to 55° C. were added and then the mixture was homogenized again for 2 minutes. The ethyl acetate was removed by evaporation at 55° C. and a reduced pressure of 200 mm. Hg whereupon water was added to the gelatin composition to make 80 ml.

35 A homogeneous dispersion was obtained which after having been stored for 24 hours at 5° C. did not at all show a crystallization tendency.

40 The gelatin composition formed could be admixed by gentle stirring with a gelatino silver halide emulsion ready for coating.

45 When in the preparation of the above dispersion the isoctadecyl alcohol and the sodium isoctadecyl sulphate were replaced by the same amounts of n-lauryl alcohol and sodium n-lauryl sulphate the color coupler soon began to crystallize on storing at 5° C.

#### EXAMPLE 2

50 1.5 g. of the color coupler of Example 1 was dissolved in a mixture of 4.5 ml. of ethyl acetate and 1.5 ml. of isoctadecyl alcohol. The solution was dispersed by means of a high-speed stirrer into 58 g. of a warm (55° C.) 10% aqueous solution of gelatin to which 3 ml. of a 10% aqueous solution of sodium isoctadecyloxypropyl sulphonate having the formula:



55 as surfactant had been added.

60 The mixture was dispersed for 2 minutes whereupon 40 ml. of water heated to 55° C. were added and homogenizing was continued for 2 minutes.

65 The ethyl acetate was removed by evaporation as described in Example 1 and water was added to make 80 ml.

70 The very stable homogeneous dispersion of particles of the alcohol containing color coupler could then be ad-



## EXAMPLE 8

Example 7 was repeated with the difference that now 0.5 g. of isoctadecyl alcohol was used instead of 0.5 g. of hydroabietyl alcohol and that the surfactant was replaced by 5 ml. of a 10% aqueous solution of sodium isoctadecyloxypropyl sulphonate.

## EXAMPLE 9

5 g. of the mask-forming compound having the formula:



were dissolved in a mixture of 30 ml. of ethyl acetate and 0.5 g. of an ethoxylated secondary synthetic C<sub>11</sub>-C<sub>15</sub> aliphatic alcohol containing 3 ethylene oxide units per molecule and commercially available for Union Carbide and Carbon under the trade name Tergitol 15-S-3, which can be represented by the formula:



in which  $x+y=8-12$ .

The solution formed was dispersed into 50 g. of a 10% aqueous solution of gelatin which was heated to 55° C. and to which had been added 5 ml. of a 10% aqueous solution of the surfactant with formula:



wherein  $x+y=8-12$ .

After having dispersed the mixture for 5 minutes, 30 ml. of hot water (50° C.) were added and homogenizing was continued for 5 minutes.

The ethyl acetate was removed by evaporation as described in Example 1 whereupon hot water was added to make 100 ml.

The dispersion formed could then be admixed by gentle stirring with a conventional red-sensitized gelatino silver halide emulsion comprising a cyan-forming color coupler.

## EXAMPLE 10

5 g. of the color coupler with formula:



were dissolved in a mixture of 30 ml. of ethyl acetate and 0.5 g. of ethoxylated secondary synthetic C<sub>11</sub>-C<sub>15</sub> aliphatic alcohol containing 9 ethylene oxide units per molecule and commercially available from Union Carbide and Carbon under the trade name Tergitol 15-S-9, which can be represented by the formula:



in which  $x+y=8-12$ .

The solution formed was dispersed into 50 g. of a 10% aqueous solution of gelatin which was heated to 55° C.

and to which had been added 5 ml. of 10% aqueous solution of the surfactant with formula:



wherein  $x+y=8-12$ .

The mixture was then further treated as described in Example 9.

The dispersion formed could then be admixed by gentle stirring with a conventional gelatino silver halide emulsion ready for coating.

## EXAMPLE 11

This example illustrates the favorable effect of the high-boiling alcohol on the viscosity of the hydrophilic colloid composition.

3 g. of the color coupler of Example 1 were dissolved in 18 ml. of ethyl acetate and 1.5 g. of isoctadecyl alcohol. The solution was dispersed in 96 g. of 10% aqueous gelatin in the presence of 4.5 ml. of 10% aqueous sodium dodecylbenzene sulphonate. The ethyl acetate was removed by evaporation as described in Example 1 whereupon 8 ml. of 10% aqueous sodium 2-heptadecenyl benzimidazole-5-sulphonate and 0.7 ml. of 10% ethanolic mucochloric acid were added. Water was added to make 225 ml. and the pH was adjusted to pH 6 by means of N sodium hydroxide.

The viscosity of the gelatin solution at 40° C. was 15 cp. and remained constant for at least 24 hours.

For comparison purposes a gelatin solution was prepared as follows.

3 g. of the color coupler of Example 1 was dissolved in 4.5 ml. N sodium hydroxide and 25.5 ml. of water.

The solution formed as well as 8 ml. of 10% aqueous sodium 2-heptadecenyl benzimidazole-5-sulphonate and 0.7 ml. of 10% ethanolic mucochloric acid were added to 96 g. of 10% aqueous gelatin. Water was added to make 225 ml. and the pH was adjusted to pH 6 by means of N succinic acid.

After having kept the gelatin solution for 1 hour at 40° C. the viscosity had increased so much that it could not be measured any more.

We claim:

1. Method of incorporating a photographic chemical adjuvant into a hydrophilic colloid coating composition for forming a water-permeable colloid layer of a photographic element according to which a solution of the said chemical adjuvant is dispersed in the said hydrophilic colloid coating composition, or is dispersed first in water or in an aqueous solution of the said water-soluble colloid and the resulting dispersion is admixed with the said hydrophilic colloid coating composition, wherein the said solution of chemical adjuvant is a solution of the adjuvant in a high-boiling substantially water-insoluble aliphatic alcohol or an ethoxylated derivative thereof corresponding to the following general formula:



wherein:

$n$  stands for 0 or 1,

$m$  stands for 0 to 30,

$R_3$  stands for hydrogen or when  $n=1$  may be alkyl, and each of  $R_1$  and  $R_2$  stands for a straight-chain or branched-chain alkyl group or together stand for the atoms necessary to close an alicyclic ring structure,  $R_1$  and  $R_2$  together comprising at least 5 C-atoms.

2. Method according to claim 1, wherein the ratio of alcohol to chemical adjuvant is in the range of 1:1 to 10:1.

3. Method according to claim 1, wherein the said alcohol is a branched-chain primary oxo-alcohol.

4. Method according to claim 1, wherein the said solution is a solution of chemical adjuvant in a mixture of the said alcohol or ethoxylated alcohol and one or more organic solvents.

5. Method according to claim 4, wherein said organic solvent is a substantially water-immiscible solvent.

6. Method according to claim 5, wherein said solvent has a solubility in water of at most 25% by weight at room temperature and a boiling point of at most 130° C.

7. Method according to claim 4, which comprises removing the said organic solvent simultaneously with or subsequently to dispersing the said solution comprising the said chemical adjuvant and the said alcohol or ethoxylated alcohol into the hydrophilic colloid coating composition, water or aqueous solution of a water-soluble colloid.

8. Method according to claim 7, wherein the said organic solvent is removed from the dispersion by evaporation.

9. Method according to claim 8, wherein the said organic solvent is removed by evaporation under reduced pressure and applying heat.

10. Method according to claim 4, wherein the ratio of alcohol to chemical adjuvant is in the range of 1:1 and 1:20.

11. Method according to claim 1, wherein the solution of the said chemical adjuvant is dispersed into the hydrophilic colloid coating composition, in water or in an aqueous solution of a water-soluble colloid in the presence of a dispersing agent.

12. Method according to claim 11, wherein said dispersing agent corresponds to the formula:



wherein

$R_1$ ,  $R_2$ ,  $R_3$ ,  $n$  and  $m$  have the same significance as in claim 1, and

$Z$  stands for the group  $-SO_3M$ ,  $-OSO_3M$ ,

$-OCO-X-SO_3M$

or  $-Y-A-SO_3M$  wherein  $M$  stands for hydrogen, an alkali metal atom, ammonium or organic ammonium,

$X$  is alkylene, aralkylene or arylene,

$Y$  is oxygen or sulphur, and

$A$  stands for an alkylene, or aralkylene group.

13. Method according to claim 11, wherein the said dispersing agent is used in an amount comprised between 2 and 30% by weight relative to the weight of chemical adjuvant.

14. Method according to claim 1, wherein the hydrophilic colloid coating composition is a photosensitive gelatino silver halide emulsion.

15. Method according to claim 14, wherein the said chemical adjuvant is a color coupler or mask-forming component.

16. Method according to claim 1 wherein the said chemical adjuvant has a solubility in water of at most 3% by weight at 20° C.

#### References Cited

##### UNITED STATES PATENTS

|    |           |         |              |       |          |
|----|-----------|---------|--------------|-------|----------|
| 30 | 2,768,894 | 10/1956 | Harriman     | ----- | 96—114.5 |
|    | 2,949,360 | 8/1960  | Julian       | ----- | 96—100   |
|    | 3,068,101 | 12/1962 | Knox et al.  | ----- | 96—114.5 |
|    | 3,617,292 | 11/1971 | Gantz et al. | ----- | 96—114.5 |

35 J. TRAVIS BROWN, Primary Examiner

U.S. CL. X.R.

96—9, 84 R, 114. 5